

## 1

3,163,504  
COMBINATION ANTI-ICING ADDITIVE  
FOR JET FUELS

Louis N. Calvino, Plainfield, N.J., assignor to Esso Research and Engineering Company, a corporation of Delaware  
No Drawing. Filed Mar. 15, 1961, Ser. No. 95,825  
7 Claims. (Cl. 44—63)

The present invention concerns hydrocarbon oil compositions, particularly jet fuels, having improved water tolerance characteristics and a process for operating jet engines utilizing said fuels. More particularly, the instant invention relates to turbojet fuel compositions having incorporated therein additives to reduce persistent haze and stable emulsions formed when such fuels containing haze promoting anti-icing additives are contacted by water.

The operating of jet engines at widely varying conditions of temperature and altitude has resulted in grave problems in regard to suitable fuel compositions to be utilized. One particularly serious problem involves the operational hazards of employing jet fuel containing dissolved and suspended water at low temperatures and at high altitudes. Jet engine aircraft are normally equipped with filters located in the fuel pumping system in order to remove suspended matter in fuel which might interfere with normal engine operation. At low temperatures and especially at the low subfreezing temperatures, such as from —45° F. to —76° F., associated with high altitudes, dissolved and suspended water in the jet fuel forms ice in the narrow passageways of the fuel flow system or on the filter surface or on the sludge layer on the filter surface. Hydrocarbons utilized as jet fuels are capable of dissolving small quantities of water from the air during normal weather, from storage tanks, and the like. Additionally, water from these sources can also become suspended in the fuel after it has become water saturated. It is this dissolved and suspended water which, upon lowering of the temperature, freezes and creates an icing problem. The formation of ice results in the creation of a considerable pressure drop in the fuel system and sometimes the complete obstruction of the fuel flow with resultant flameout and loss of the aircraft.

In order to alleviate this critical problem, anti-icing additives have been incorporated into jet fuel compositions to allow operation of the aircraft at low temperatures without excessive ice formation. These additives have usually been aliphatic oxygen-containing compounds having from about 1 to 30 carbon atoms per molecule. Typical anti-icing compounds utilized in the past have included ether alcohols, such as alkoxy alkanols formed by the reaction of ethylene oxide or propylene oxide with aliphatic alcohols, for example, ethanol and the like, to yield compounds such as 2-methoxyethanol, 2-ethoxyethanol and the like; alcohols, such as alkanols, for example, methanol, ethanol, isopropanol, and the like; glycols, such as alkanediols, like ethylene glycol, propylene glycol, hexylene glycol, and the like; polyalkylene glycols, such as polyethylene glycol and the like; alkanol amines, such as aminomethyl propanol and the like; ethers, such as alkyl ethers, like isopropanol ethers, and alkoxy alkanol ethers, such as bis(2-methoxyethyl)ethers; ether esters, such as alkoxy alkanol esters of low molecular weight monocarboxylic acids, such as 2-methoxyethyl acetate and the like. These additives and combinations thereof are particularly useful as anti-icing additives

## 2

and in general are set forth in U.S. Patents 2,952,121, 2,701,754, 2,840,461, 2,722,099, 2,668,522, 2,599,338 and so forth.

Although these additives have generally helped to alleviate the icing effects by function as freezing point depressants or surfactants they have created a new and serious problem. In general, these anti-icing additives all exhibit a pronounced tendency to suspend water with which the hydrocarbon fuel comes in contact and to yield stable oil-in-water emulsions and persistent aqueous haze formations. Thus, these additives, particularly the aliphatic glycols of from 6 to 21 carbon atoms per molecule, and additive anti-icing combinations containing these glycols have a particular tendency to promote aqueous haze conditions when jet fuel containing these additives contacts water. The formation of persistent aqueous haze or stable water-in-oil emulsions in these fuels may adversely affect the performance of these fuels under severe operating conditions. Additionally, these stable emulsions induce corrosion and in general affect the appearance, marketability, and consumer acceptance of the petroleum product. Since water exists in most storage tanks, pipelines, and other container vessels during the handling, transportation and storage of the fuel, haze formation and emulsions are also impossible to avoid.

It is, therefore, an object of this invention to reduce the tendency of hydrocarbon oils containing haze-promoting anti-icing additives from forming persistent haze or stable emulsions when contacted with water. A further object is to promote the marketability and appearance of jet fuels by reducing the tendency of these fuels containing aliphatic oxygen anti-icing additives to form aqueous haze conditions. Further objects and benefits are apparent to those skilled in the art in light of the instant disclosures.

The applicant has discovered that the incorporation into hydrocarbon oil compositions of a minor amount of an alkyl pyrrolidone destabilizes and inhibits aqueous haze formation and water-in-oil emulsions induced by haze-promoting anti-icing additives. It has been found that these alkyl pyrrolidones are particularly effective in jet fuel compositions containing aliphatic oxygen-containing anti-icing additives of from 1 to 30 carbon atoms. More particularly, the N-alkyl pyrrolidones have been found to be especially effective in reducing aqueous haze induced by aliphatic glycols. The pyrrolidones of this invention may be incorporated into the hydrocarbon oil either before or after the contacting of water by the said oil. These pyrrolidones may be utilized in combination with the anti-icing additives in a concentrate form or added singly into the hydrocarbon oil. The pyrrolidones suitable for the purposes of this invention include those alkyl substituted pyrrolidones wherein the alkyl radical has from 1 to 4 carbon atoms. Preferred due to their efficacy are N-alkyl pyrrolidones, while especially preferred by reason of commercial availability and performance are the N-alkyl-2-pyrrolidones, such as N-methyl-2-pyrrolidone.

It should be noted that the employment of pyrrolidone itself is not suitable for the purposes of this invention due to its restrictive and limited solubility in hydrocarbon oils. The applicant has found that his inventive compounds exhibit a suitable solubility balance such that effective dehazing is accomplished. The quantity of the inventive pyrrolidones required to be utilized depends to some extent on the particular anti-icing additive employed and its concentration level. Usually minor amounts of pyrrol-

idones are effective, i.e. from about 0.01 to 2.0% by volume, with from 0.1 to 1.0% by volume normally effective. The ratio of anti-icing additive to the pyrrolidones ranges from 1/10 to 5/1, with from 1/4 to 2/1 particularly effective. The anti-icing additives are usually incorporated in minor amounts sufficient to give the effective anti-icing protection desired. These amounts commonly range from 0.001% by volume to about 3.0% by volume, with from 0.05% to about 1.5% by volume the most common amount employed.

Suitable pyrrolidones for the purposes of this invention include the following: 3-methyl-N-methyl-2-pyrrolidone, 4-ethyl-N-ethyl-2-pyrrolidone, N-ethyl-3-pyrrolidone, 3,4-dimethyl-N-methyl-2-pyrrolidone, N-methyl-2-pyrrolidone, N-propyl-2-pyrrolidone, and the like.

The commonly employed glycols include those alkyl glycols having from 2 to 21 carbon atoms per molecule, such as the mono, di, tri and higher glycols of ethylene, propylene, isobutylene, and the like, and especially those alkyl diols characterized by having an alkyl radical directly attached to at least one of the carbon atoms to which a hydroxyl group is attached. The alkyl group may contain from 1 to 4 carbon atoms, although it is preferred that the alkyl group be a methyl group. Among the preferred diols, those having from 6 to 8 carbon atoms are most preferred, particularly the alkyl glycols as the hexylene glycols, as, for example, 2-methyl-2,4-pentanediol, and hexanediol-2,5. Especially preferred among the hexylene glycols is 2-methyl-2,4-pentanediol.

The hydrocarbon oils in which the additives of this invention may be incorporated are those hydrocarbon fuels boiling between about 250° F. and 750° F. and particularly those liquid petroleum turbojet fuels boiling in the range between about 300° F. and 550° F. These fuels include those used to power turboprop, turbofan, ramjet, pulsejet and similar jet engines. These fuels normally contain at least 10% by volume of paraffinic components and meet ASTM Specification for Aviation Turbine Fuels D-1655-59T. These fuels are additionally defined by Military Specifications MIL-J-5161E (ASG), MIL-J-5624E, MIL-F-25524A (USAF), and the like, and are generally referred to as JP-4, JP-5, and JP-6. The inventive additives may also be incorporated into heating oils, diesel oils, transformer oils, turbine oils, lubricating oils, and the like containing aliphatic oxygen-containing additives which promote the formation of a persistent aqueous haze condition when contacted with water. Diesel fuels are as described in ASTM Specification D-975-53T, while heating oils are described in ASTM Specification D-396-48T, particularly those in Grades 1 and 2 thereof. These fuels, in addition to the anti-icing and inventive additives, may include rust inhibitors, antistatic additives, corrosion inhibitors, dyes, dye stabilizers, polymeric additives, and the like.

The persistence of the haze formed in oil upon contact with water is measured in Waring Blender Haze Tests wherein five milliliters of water and 500 milliliters of the oil, such as JP-4, with and without haze promoting additives are mixed in a Waring Blender for a period of one minute; the oil-water mixture is then observed over a specified time period. The amount of light which is transmitted through the oil under standardized conditions is measured, or the haze and emulsification conditions of the fuel are visibly observed during this time period. Where measured, the light transmission is expressed as a percentage of the total light emitted from the source. These test methods have been found to be an extremely effective means for determining the degree to which haze is present in hydrocarbon oils.

The effectiveness of the present inventive combination may be ascertained by the following examples.

#### EXAMPLE 1

The Waring Blender test as described was conducted using a JP-4 jet fuel containing a well known commercial

anti-icing additive of hexylene glycol, i.e. 2-methyl-2,4-pentanediol. The results obtained are as indicated in Table I.

5 DEHAZING JET FUEL (JP-4) CONTAINING AN ANTI-ICING ADDITIVE

| 10 | Additive                                                | Percent Light Transmission |      |      |       |       |       |       |
|----|---------------------------------------------------------|----------------------------|------|------|-------|-------|-------|-------|
|    |                                                         | Time in Hours After Mixing |      |      |       |       |       |       |
|    |                                                         | 0.5                        | 1    | 2    | 3     | 4     | 5     | 6     |
| 15 | JP-4 Fuel                                               | 92                         | 95   | 98.5 | 99.5  | 100   | ----- | ----- |
|    | JP-4+0.25% hexylene glycol                              | 85                         | 89   | 95   | 98    | 99    | 99.5  | 100   |
| 20 | JP-4+0.25% N-methyl-2-pyrrolidone                       | 90                         | 93   | 97.5 | 99.5  | 100   | ----- | ----- |
|    | JP-4+0.25% hexylene glycol+0.25% N-methyl-2-pyrrolidone | 90                         | 93   | 97.5 | 98.5  | 99.5  | 100   | ----- |
| 25 | JP-4+0.25% hexylene glycol+1.0% N-methyl-2-pyrrolidone  | 99                         | 99.5 | 100  | ----- | ----- | ----- | ----- |
|    | JP-4+0.25% Additive X <sup>1</sup>                      | 82                         | 87   | 90   | 96    | 97    | 99.5  | 100   |
| 30 | JP-4+0.25% Additive X+0.25% N-methyl-2-pyrrolidone      | 89                         | 93   | 97   | 100   | ----- | ----- | ----- |

<sup>1</sup> Note—is a mixture of 67% hexylene glycol+33% 2-methoxyethanol.

The above results indicate the remarkable effectiveness with which the alkyl pyrrolidones eliminate stable haze conditions caused in hydrocarbon oil compositions by the presence of well known haze-promoting anti-icing additives, such as hexylene glycol and mixtures of hexylene glycol with alkoxy alkanols. The anti-icing additives employed are those commonly accepted as effective anti-icing additives for incorporation in jet fuels for operating jet engines at subfreezing temperatures.

35 The results achieved by the alkyl pyrrolidones are rendered completely unexpected in that the use of N-methyl-2-pyrrolidone alone in JP-4 slightly increased the the haze in the JP-4 over the fuel without any additive.

#### EXAMPLE 2

To a turbojet engine fuel designated JP-4 and meeting the military and ASTM requirements set forth is added about 0.2% by volume of 2-methyl-2,4-pentanediol and 0.1% by volume of 2-methoxyethyl acetate to produce a fuel composition appropriate for use at subfreezing temperatures. The addition of about 0.25% by volume of 3-methyl-N-methyl-2-pyrrolidone improves the water tolerance characteristics of said fuel without unduly affecting its anti-icing characteristics.

#### EXAMPLE 3

The water tolerance properties of a turbojet engine fuel boiling between about 275° F. and about 480° F. and containing 0.3% by volume of isopropanol and about 0.2% by volume of 2-methyl-2,4-pentanediol is considerably improved by the addition of about 0.5% by volume of N-ethyl-2-pyrrolidone.

#### EXAMPLE 4

60 Aqueous haze clearance is promoted by the addition of about 2.0% by volume of N-methyl-3-pyrrolidone to a heating oil boiling in the range between 324° F. and 645° F. and consisting of more than 10% by volume of catalytically cracked stock and containing about 1.0% by volume of isopropanol.

#### EXAMPLE 5

A turbojet fuel (JP-4) containing about 0.2% by volume of 2-methoxy ethanol and forming a stable oil-in-water emulsion when contacted with water is effectively demulsified by the incorporation of about 0.1 volume percent of 3,3-dimethyl-N-methyl-2-pyrrolidone.

From the foregoing examples, the remarkable effectiveness of alkyl pyrrolidones in reducing aqueous haze formation in hydrocarbon oils is demonstrated. The re-

sults are particularly surprising wherein additives tending to stabilize oil-in-water emulsions are dehazed by the addition of N-methyl-2-pyrrolidone. The effectiveness of the additives of this invention permits a significant improvement in the marketability, appearance, and water tolerance properties of petroleum products and simplifies the handling and the storage of such products.

What is claimed is:

1. A liquid hydrocarbon fuel boiling in the range of about 250° F. to 750° F. containing an alkyl diol having 2 to 21 carbon atoms per molecule additive in sufficient quantity to provide anti-icing protection and in sufficient quantity to promote the formation of an aqueous haze when said fuel is contacted with water; said fuel also containing a minor amount sufficient to dehaze said fuel of an N-alkyl pyrrolidone.

2. A composition as claimed in claim 1 wherein said fuel is a turbojet engine fuel boiling in the range between 300° F. and 550° F.

3. A composition as claimed in claim 1 wherein said N-alkyl pyrrolidone has from 1 to 4 carbon atoms in the alkyl radical.

4. A composition as claimed in claim 1 wherein said minor amount is a concentration of from about 0.01% by volume to about 2.0% by volume.

5. A liquid hydrocarbon fuel boiling in the range between 300° F. and 550° F. containing an alkyl diol hav-

ing 2 to 21 carbon atoms per molecule in sufficient quantity to overcome icing effects and which is sufficient to promote the formation of an aqueous haze when said fuel is contacted with water and to which has been added from about 0.2% to 1.0% by volume of a N-alkyl pyrrolidone wherein the alkyl radical has from 1 to 3 carbon atoms.

6. A composition as defined by claim 5 wherein said alkyl diol is 2-methyl-2,4-pentanediol.

7. A composition as claimed in claim 5 wherein said N-alkyl pyrrolidone is N-methyl-2-pyrrolidone and wherein said alkyl diol is hexylene glycol.

References Cited in the file of this patent

UNITED STATES PATENTS

|           |                  |              |
|-----------|------------------|--------------|
| 2,550,981 | Eberz -----      | May 1, 1951  |
| 2,550,982 | Eberz -----      | May 1, 1951  |
| 2,701,754 | Haworth -----    | Feb. 8, 1955 |
| 2,722,099 | Wasserbach ----- | Nov. 1, 1955 |

FOREIGN PATENTS

|           |               |               |
|-----------|---------------|---------------|
| 1,020,209 | Germany ----- | Nov. 28, 1957 |
|-----------|---------------|---------------|

OTHER REFERENCES

25 German application 1,094,037/(Kl. 46a67), Dec. 1, 1960.